

## UNITED STATES PATENT OFFICE

ALBERT RUSSELL CAMPBELL, OF COVINGTON, KENTUCKY, ASSIGNOR OF FORTY-NINE PER CENT TO DAVID RUBIN, OF CINCINNATI, OHIO

## WATERPROOFING COMPOUND FOR CEMENT AND CONCRETE

No Drawing.

Application filed November 17, 1927. Serial No. 234,041.

The invention disclosed herein makes it possible to utilize to advantage by-products that have heretofore been considered waste products and at the same time provide a new composition that is very efficient and effective as a waterproofing agent for cement, concrete, mortar and the like.

In addition to the fact that the herein disclosed invention functions as a waterproofer, it also operates as a hardener for cement, concrete, mortar and other similar substances.

In the molding of various articles, especially iron and steel articles, a certain type of sand is used that is generally referred to as molder's sand or foundry sand. This sand will vary somewhat in its composition. The variation or exact composition of the indicated sand is not, however, material. In the process of molding, portions of the mold or sand are subjected to extremely high temperatures, various gases are either formed or thrown off and these gases in some manner affect the sand of the mold, and various fine parts of the iron and steel become separated from the casting and mingle with the sand of the mold. The sand when taken from the mold is used repeatedly until it reaches a condition such that it can no longer be used for molding. At or about that time the sand may be properly referred to as burnt sand. This sand is used in preparing the composition of the invention.

The castings taken from the sand are generally ground to some extent on a carborundum wheel with the result that some of the carborundum and some of the iron becomes a by-product, or waste product. It has been the practice around foundries and the like to take this carborundum and the waste iron and to throw it with the burnt sand, all of which was considered of no further value.

The invention herein consists in the taking of the aforesaid burnt sand, iron and carborundum, and admixing therewith a quantity of salt. The resultant product when added to cement mixtures and the like has been found to render the resultant mass of concrete, cement, et cetera, to such low water absorption properties that the indicated structure may be said to be substantially wa-

terproof. It has also been found that the hardness of the structure is materially increased.

An analysis of the compound shows substantially the following composition:

|             | Per cent |
|-------------|----------|
| Ground iron | 8        |
| Carborundum | 2 1/4    |
| Salt        | 1        |
| Burnt sand  | 88 3/4   |

Analyses of various sands used in making batches of waterproofing compound, and all of which batches proved satisfactory and efficient, were as follows:

|         | Iron     | Burnt silica | Carbo-rundum |
|---------|----------|--------------|--------------|
|         | Per cent | Per cent     | Per cent     |
| Batch 1 | 2.52     | 95.43        | 2.00         |
| Batch 2 | 1.90     | 98.00        | .03          |

To the foregoing batches there was added approximately sufficient salt to make the salt content of the resultant composition approximately 1% thereof.

A second mixture of the following proportions was made, tested and found to give the indicated results:

|                       | Per cent |
|-----------------------|----------|
| Portland cement       | 50       |
| Ground iron           | 7 1/2    |
| Carborundum           | 1 1/2    |
| Salt                  | 1        |
| Burnt molder's sand   | 25       |
| Unburnt molder's sand | 15       |

To 100 pounds of the foregoing composition there was added 100 pounds of clean sharp sand and sufficient water to mix same. The resultant product attained the indicated results. The foregoing composition can be used as a cement surfacing for substantially waterproofing the understructure upon which the surfacing is applied. If desired the waterproofing compound may be admixed with a concrete mass or the like, thereby rendering such concrete mass substantially free of water absorption and also to give greater hardness to the mass.

In instances where the composition was added to plaster, brick mortar and tile mortar, analogous results were obtained. Although there would naturally be some variation in the composition of mortars, cement, concrete masses and the like, substantially uniform results are obtained in each instance dependent upon the quantity of the waterproofing compound used in the mixture. If approximately a quantity of waterproofing equivalent to the quantity of cement is employed in a given batch, a very effective waterproofing is attained. If the quantity of waterproofing substance is decreased, of course the degree of possible water absorption becomes greater.

What is claimed is:

1. A waterproofing compound comprising substantially 95% burnt silica, 2% iron, 2% carborundum and 1% salt.
2. The combination with a hydraulic cementitious material of a compound comprising substantially 95% burnt silica, 2% iron, 2% carborundum and 1% salt.

25 In testimony whereof, I have hereunto subscribed my name this 14th day of November, 1927.

ALBERT RUSSELL CAMPBELL.

30

35

40

45

50

55

60

65